

# UNITED STATES PATENT OFFICE.

EDGAR A. CUSTER, OF PHILADELPHIA, PENNSYLVANIA, ASSIGNOR TO THE CUSTER SANDLESS CASTING COMPANY, OF PHILADELPHIA, PENNSYLVANIA, A CORPORATION OF DELAWARE.

## NON-ANNEALED CAR-WHEEL.

1,022,723.

Specification of Letters Patent.

Patented Apr. 9, 1912.

No Drawing.

Application filed December 12, 1910. Serial No. 596,926.

To all whom it may concern:

Be it known that I, EDGAR A. CUSTER, a citizen of the United States, residing in the city of Philadelphia, in the State of Pennsylvania, have invented certain new and useful Improvements in Non-Annealed Car-Wheels, of which the following is a specification.

My invention relates to wheels of any size and section, and particularly to car wheels, and the invention consists in producing an integral cast iron non-annealed wheel which may be used as cast and which does not require any annealing process whatsoever, but which shall have a chilled tread and a homogeneous body free from shrinkage strains of relatively soft and machinable metal.

My improved car wheel may be of any standard size or design, and is preferably cast in a permanent mold of any desired construction, which will permit parts of the mold to be withdrawn from contact with the casting as desired. Consequently the parts of the mold forming the hub and spokes of the casting may be withdrawn as soon as the metal has set, but the parts of the mold which are in contact with the tread and flange may be permitted to remain in position for a longer period of time, and until the metal in the tread and flange has been chilled.

Preferably the molten metal is rapidly cooled and is brought swiftly to the point of setting almost simultaneously throughout all portions of the casting in contact with the mold. Thereupon the parts of the mold in contact with any portion of the casting which it is desired to make machinable such as the hub, spokes, plates or inner portion of the rim are withdrawn or separated from the casting, which interrupts or delays the cooling of such portions of the casting. The cooling of the portions of the wheel which it is desired to chill, such as the tread and flange, is continued rapidly, however, until such portions are chilled to the desired depths. This is accomplished by making the parts of the mold adjacent to such portions of the wheel relatively thick in section, thus providing a large heat-absorbing capacity in the mold adjacent to such portions of the wheel. Preferably also the parts of the mold adjacent to the tread and flange of the wheel are kept at a rela-

tively low temperature, so that the heat will be absorbed very quickly from the cooling metal. Preferably the temperature of the mold adjacent to the portions of the wheel which it is desired to chill deeply is not permitted to rise above 600° F. 60

By causing the molten metal to set almost simultaneously throughout the casting and promptly withdrawing or separating parts of the mold from certain portions of the casting such as the hub, spokes or plates or the inner portion of the rim, the casting will be free from shrinkage strains and all tendency of the casting to pull apart will be avoided and the wheel, except the tread and flange, will consist of homogeneous metal. 70

In my improved construction the body of the wheel is of homogeneous material of very fine grain throughout, which can be easily machined and is free from shrinkage strains. The tread, however, is chilled and contains the characteristic white crystals of chilled iron. Consequently no annealing process is necessary as the wheel is ready for use as it comes from the mold with a machinable hub and a chilled tread. 80

I claim as my invention:

1. An integral cast iron non-annealed wheel having a chilled tread and homogeneous body free from shrinkage strains with a center comprising machinable metal. 85

2. An integral cast iron non-annealed wheel having a chilled tread and homogeneous body, free from shrinkage strains, with a center comprising soft metal having a fine grain. 90

3. An integral cast iron non-annealed wheel having a chilled tread and having its hub, spokes and rim free from shrinkage strains and of machinable metal. 95

4. An integral cast iron non-annealed wheel free from shrinkage strains having portions of homogeneous machinable metal of fine grain throughout and having portions of chilled iron containing white crystals. 100

5. An integral cast iron non-annealed wheel free from shrinkage strains having its hub, spokes and rim of homogeneous machinable metal of a fine grain throughout, and having its flange and tread of chilled iron containing white crystals. 105

6. An integral cast iron non-annealed wheel produced in a permanent mold which 110

causes the molten metal to set swiftly almost simultaneously throughout, said wheel having a homogeneous body free from shrinkage strains with a center of machinable metal.

7. An integral cast iron non-annealed wheel produced in a permanent mold which causes the molten metal to set swiftly simultaneously throughout, said wheel having a

homogeneous body free from shrinkage strains with a center of machinable metal, and having a flange of harder metal.

This specification signed and witnessed this 1st day of December, A. D., 1910.

EDGAR A. CUSTER.

Signed in the presence of—

AMBROSE L. O'SHEA,  
HELEN M. DAMES.